

## UNITED STATES PATENT OFFICE

2,613,161

## FLUID GASKET SEALING COMPOSITION

Chester M. White, Rochester, N. Y., assignor to  
Genesee Research Corporation, Rochester,  
N. Y., a corporation of New York

No Drawing. Application September 17, 1947,  
Serial No. 774,680

3 Claims. (Cl. 106—220)

1

The present invention relates generally to the art of stabilizing castor oil and its derivatives and is more particularly concerned with the production of stabilized castor oil, blown castor oils of various consistencies, and acetylated castor oil, or stabilized mixtures of any of these oils.

Workers in the art of castor oil use are familiar with the problem of so-called "gumming" or "setting up" of castor oil and its derivatives upon standing. For many uses of castor oil this has been and still is a serious problem, as will be more particularly pointed out hereinafter. Just what causes castor oil or its derivatives to gum or set up is not entirely known but the fact remains that when these oils are allowed to stand for any time they gradually thicken to a point where they refuse to flow and finally become hard and unworkable. The gumming or setting up is probably due to polymerization, although it may well be the result of oxidation. It is perhaps a combination of the two but, be that as it may, the present invention is limited in no way to the actual cause of the gumming or setting up.

It is, accordingly, one of the salient features and primary objects of the present invention to stabilize castor oil, whether of the cold or hot pressed variety, as well as blown castor oils of various consistencies and acetylated castor oil or mixtures thereof.

It is also an object of the invention to produce several compositions of matter employing the stabilized oils of the invention where oil stability is particularly critical.

The foregoing and other objects of the invention are achieved through the very simple expedient of merely adding to the oils a small percentage of potassium hydroxide (KOH), thus to form in the oils in situ a potassium soap. It has been found that this in situ formation of a small amount of potassium soap serves effectively to stabilize castor oil and its derivatives and inhibit gum formation and setting up through standing. Stated differently, the in situ formation of a small amount of potassium soap in the oils serves to inhibit polymerization and/or oxidation of the oils, resulting in gumming or setting up.

Potassium soap is formed merely by adding to the castor oil or its derivatives or mixtures there-

of, a small amount of KOH in the form of solid 90% KOH, although it is understood, of course, that the small amount of KOH could be, and usually is, added in a solvent medium such as water or an organic solvent, such as a glycol or an alcohol-ether mixture.

The amount of KOH added to provide in situ formation of potassium soap depends upon the character of the oil, i. e., whether it is ordinary castor oil, acetylated castor oil or whether it is a blown castor oil. It has been observed that as the extent of blowing the castor oil is increased more soap is required to prevent the oil from setting up. In every case there is a minimum 15 of soap content which will be effective to render the oil stable and likewise in every case there is a maximum soap content above which the soap crystallizes from the oil or forms a gel which prevents the oil from flowing. In the case of blown castor oil, the optimum soap range becomes shorter as the extent of blowing increases. Both ordinary castor oil and acetylated castor oil require, generally speaking, less potassium soap than blown castor oil. There is, however, a maximum soap content above which ordinary castor oil and acetylated castor oil tend to set up. It has been found that with the various 20 grades of castor oil and castor oil derivatives one must use at least 0.1% KOH as a minimum to effect in situ formation of sufficient potassium soap to inhibit gelling or setting up. With all 25 grades of oil there is a maximum of 1.0% KOH since above this point the in situ-formed soap will be present in an amount sufficient to crystallize from the oil or to form a gel which prevents the oil from flowing.

The foregoing minimum and maximum KOH additions have been determined experimentally. There has been added to castor oil and several 30 of its derivatives various percentages of potassium hydroxide which produced corresponding percentages of soap. The samples were placed in an oven, maintained at 210° F. and these were examined every day and the flow of the samples 35 was noted. Data on several castor oils and castor oil derivatives, indicating maximum and minimum KOH addition, is given in the following table:

| Grade of oil                   | Soap content (based on added KOH) |          |
|--------------------------------|-----------------------------------|----------|
|                                | Minimum                           | Maximum  |
| P-8 Acetylated Castor Oil..... | 0.1% KOH                          | 1.0% KOH |
| #1 Castor Oil.....             | 0.2% KOH                          | 1.0% KOH |
| #300 Blown Castor Oil.....     | 0.4% KOH                          | 1.0% KOH |
| #900 Blown Castor Oil.....     | 0.5% KOH                          | 1.0% KOH |
| #1200 Blown Castor Oil.....    | 0.6% KOH                          | 1.0% KOH |
| #30 Blown Castor Oil.....      | 1.0% KOH                          | 1.0% KOH |

## PHYSICAL PROPERTIES

| Property                   | Min.   | Ave.   | Max.   | Property    | Temp. (approx.)   |
|----------------------------|--------|--------|--------|-------------|-------------------|
| Density @ 15° C. (lb./gal) | 8.03   | 8.07   | 8.16   | Flash Point | 293° C.           |
| Sp. Gr. @ 15° C./4° C      | .966   | .971   | .976   | Fire Point  | 316° C.           |
| Ref. Index @ 25° C         | 1.4680 | 1.4685 | 1.4690 | Pour Point  | -35° C.           |
| Color (Lovibond)           | 10Y    | 15Y    | 20Y    | Viscosity   | (40° C., 91.0 cp. |
| Volatile Matter percent    | 0      | .75    | 1.50   | (C. G. S.)  | 70° C., 32.5 cp.  |
| Ash                        |        | trace  |        |             | 100° C., 12.8.    |

In general, the amount of potassium soap formed in the oil will approximate five times the amount by weight of added KOH. Thus, the minimum soap content will be 0.5% and the maximum soap content 5.0%.

The various castor oils which may be stabilized in accordance with the present invention are identified by the following physical and chemical properties:

## Specifications of #30 castor oil

Chemical composition: Processed castor oil.  
General appearance: Bright, clear, viscous liquid, free from moisture and suspended matter.

## PHYSICAL PROPERTIES

|                            |        |
|----------------------------|--------|
| Density @ 15° C. (lb./gal) | 8.55   |
| Sp. gr. @ 15° C./4° C      | 1.025  |
| Ref. index @ 25° C         | 1.4851 |
| Color (G. H.)              | 13     |
| Volatile matter (percent)  | 0.20   |
| Pour point (°F.)           | 141    |
| Flash point (°C.)          | 218    |
| Fire point (°C.)           | 307    |
| Viscosity:                 |        |
| Engler @ 100° C            | 3000   |
| SUS @ 210° F               | 2165   |

## CHEMICAL PROPERTIES

|              |     |
|--------------|-----|
| Acid value   | 15  |
| Iodine value | 52  |
| Sap. value   | 210 |

## SOLUBILITY

|                        |    |
|------------------------|----|
| Water                  | I  |
| Alcohols:              |    |
| Cold                   | PS |
| Hot                    | S  |
| Esters                 | S  |
| Ketones                | S  |
| Ethers                 | S  |
| Aliphatic hydrocarbons | PS |
| Aromatic hydrocarbons  | S  |

I—insoluble.

S—soluble.

PS—partly soluble.

## Specifications P-8 castor oil

Chemical composition: Glyceryl-tri-aceto-ricinoleate.

General appearance: Bright, clear and free from moisture and suspended matter.

## CHEMICAL PROPERTIES

| Property               | Min. | Ave. | Max. |
|------------------------|------|------|------|
| Acid Value             | .2   | 2.0  | 4.0  |
| F. F. A. (1% as Oleic) | .10  | 1.0  | 2.0  |
| Acetyl Value           | 147  | 150  | 154  |
| Iodine Value           | 72   | 75   | 78   |
| Sap. Value             | 290  | 297  | 305  |
| Unsaponifiable percent | .25  | .50  | .75  |
| Hehner Value           | 94   | 95   | 96   |

## 20 SOLUBILITY

|                        |                            |
|------------------------|----------------------------|
| Water                  | Insoluble.                 |
| Alcohol                | Partly soluble to soluble. |
| Esters                 | Soluble.                   |
| Ketones                | Soluble.                   |
| Ethers                 | Soluble.                   |
| Aliphatic hydrocarbons | Soluble.                   |
| Aromatic hydrocarbons  | Soluble.                   |

## Typical analysis of #300 castor oil

Chemical composition: Processed castor oil.  
General appearance: Bright, clear, and free from moisture and suspended matter.

## PHYSICAL PROPERTIES

|                                  |        |
|----------------------------------|--------|
| Color (G. H.)                    | 10     |
| Ref. index, 25° C                | 1.4813 |
| Sp. Gr., 15° C                   | .994   |
| Viscosity (Engler secs. 100° C.) | 313    |

## CHEMICAL PROPERTIES

|                             |       |
|-----------------------------|-------|
| F. F. A. (percent as oleic) | 2.1   |
| Acid value                  | 4.2   |
| Iodine value                | 81.8  |
| Sap. value                  | 191.3 |

## 50 Specifications of #900 castor oil

|              |                  |
|--------------|------------------|
| Acid value   | Under 11         |
| Iodine value | 75 (approximate) |

|                            |                 |
|----------------------------|-----------------|
| Refractive index           | 1.4827 @ 20° C. |
| Specific gravity @ 15° C.: |                 |

|      |       |
|------|-------|
| Min. | 0.990 |
| Ave. | 0.995 |
| Max. | 0.998 |

|                    |                 |
|--------------------|-----------------|
| Viscosity @ 100° F | 10,000 S. U. V. |
| Viscosity @ 210° F | 260 S. U. V.    |

## 60 Specifications of #1 castor oil

General appearance: Bright, clear, and free from moisture and suspended matter.

## PHYSICAL PROPERTIES

| Property                | Min.   | Ave.   | Max.   | Property          | Temp. (approx.)    |
|-------------------------|--------|--------|--------|-------------------|--------------------|
| Sp. Gr. @ 15.5° C./4° C | .958   | .959   | .962   | Melting Point     | -10° C. to -18° C. |
| Ref. Inc. @ 25° C       | 1.4470 | 1.4775 | 1.4780 | 25° C., 675. cp.  |                    |
| Color (Lovibond)        | 2.0Y   | 3.0Y   | 4.0Y   | 40° C., 250. cp.  |                    |
| Volatile Matter percent | .20    | .30    | .50    | 70° C., 50. cp.   |                    |
| Ash                     |        | trace  |        | 100° C., 16.9 cp. |                    |

## CHEMICAL PROPERTIES

| Property                    | Min. | Ave. | Max. |
|-----------------------------|------|------|------|
| Acid Value                  | .40  |      | 4.0  |
| F. F. A. (as Oleic) percent | .20  |      | 2.0  |
| Acetyl Value                | 147  | 150  | 154  |
| Iodine Value                | 82   | 83   | 88   |
| Sap. Value                  | 176  | 180  | 183  |
| Hehner Value                | 94   | 95   | 96   |
| Reichert Meissl Value       | .20  | .25  | .30  |
| Unsaponifiable percent      | .25  | .39  | .50  |

An important use for the stabilized castor oils of the present invention is in adhesive or cementing compositions having an enhanced adhesive tenacity, especially to metal surfaces. Cementing compositions may be prepared, employing the stabilized castor oils of the invention, which are of liquid consistency and which remain soft and pliable so that the seal may be broken. By remaining liquid in consistency, through the virtue of castor oil stabilization, the cementing composition may be applied by means of a brush.

Employing the stabilized castor oils one may produce a cementing composition which forms films which are flexible, durable and inordinately resistant to water and many organic solvents both at low and moderately high temperatures. Cementing compositions of this character find particular utility in automotive use, such as gasket cements.

Preferably, the stabilized castor oil or castor oil derivative forms the basis for the cementing or sealing composition and mixed therewith are rosin, solvents and fillers. Illustrative of a liquid cementing or sealing composition containing the stabilized castor oil or derivatives is the following:

49-55% blown castor oil (#40)

1.15%-4.60% KOH (45%)

8-12% rosin

14-17% solvents

17-23% fillers

As stated, the castor oil in the foregoing formulation may be ordinary castor oil or it may be blown or acetylated castor oil, or various mixtures thereof. When ordinary castor oil and acetylated castor oil are employed, less KOH is necessary.

Rosin is preferred in the composition, although other natural or synthetic resinous materials could be employed, such as the well-known vinyl, alkyd and melamine resins. With respect to this resinous constituent, increase over the percentage range indicated might cause hardening on exposure to high temperature, while decrease in the range will not give sufficient tackiness to the composition. Various low-boiling solvents or mixtures thereof may be employed such as acetone, methyl alcohol, ethyl alcohol, propyl alcohol, etc., although a mixture of acetone and methyl alcohol is preferred.

Any convenient filler or mixture of fillers may be employed such as asbestos pulp, talc, kaolin, calcium carbonate, magnesia, kieselguhr, mica and lampblack. Mica and lampblack are preferred.

In the preparation of the cementing composi-

tion, it is preferable to add the KOH to the castor oil, dissolved in solvents, and then heat slightly. After heating the fillers may be added and the mixture stirred until uniform consistency is reached.

Falling specifically within the foregoing general formulation of cementing composition is the following example:

52.00% #40 castor oil (blown) } free oil and soap  
1.25% KOH (45%) }  
10.00% rosin }  
8.00% acetone }  
8.15% methyl alcohol } solvents  
9.30% aratone 270 (mica) }  
9.30% mica C-3000 } fillers  
2.00% lampblack }

This formulation provides a particularly useful liquid gasket sealing composition which may be applied by means of a brush.

What is claimed is:

1. A fluid gasket sealing composition having approximately the following formula:

|                        | Per cent  |
|------------------------|-----------|
| Blown castor oil       | 49-55     |
| KOH (45%)              | 1.15-4.60 |
| 25 Rosin               | 8-12      |
| Solvents (low-boiling) | 14-17     |
| Fillers                | 17-23     |

2. A fluid gasket sealing composition having approximately the following formula:

|                    | Per cent |
|--------------------|----------|
| Blown castor oil   | 52.00    |
| KOH (45%)          | 1.25     |
| Rosin              | 10.00    |
| 35 Acetone         | 8.00     |
| Methyl alcohol     | 8.15     |
| Aratone 270 (mica) | 9.30     |
| Mica C-3000        | 9.30     |
| Lampblack          | 2.00     |

40 3. A fluid gasket sealing composition consisting essentially of 8-12% of a resinous material, 17-23% of a filler, 14-17% of a low-boiling solvent and a base consisting essentially of 49-55% of a non-esterified oil selected from the group consisting of castor oil, blown castor and acetylated castor oil and 1.15% to 4.60% of added KOH (45%), said oil, by virtue of the presence of in situ formed potassium soap, being fluid and flowable and effectively stabilized against gumming and setting-up characteristic of untreated oil.

CHESTER M. WHITE.

## REFERENCES CITED

55 The following references are of record in the file of this patent:

## UNITED STATES PATENTS

| Number       | Name             | Date          |
|--------------|------------------|---------------|
| 1,883,270    | Hipple           | Nov. 22, 1932 |
| 60 2,066,958 | Brownback        | Jan. 5, 1937  |
| 2,217,723    | Benoit           | Oct. 15, 1940 |
| 2,305,228    | Woodhouse et al. | Dec. 15, 1942 |
| 2,327,450    | Parker           | Aug. 24, 1943 |
| 2,337,650    | Dolian           | Dec. 28, 1943 |
| 65 2,345,585 | Clark et al.     | Apr. 4, 1944  |
| 2,382,931    | Woodhouse et al. | Aug. 14, 1945 |
| 2,420,127    | Doelling         | May 6, 1947   |
| 2,517,044    | Smith            | Aug. 1, 1950  |